

# United States Patent [19]

Allard et al.

[11] 3,903,058

[45] Sept. 2, 1975

[54] **PROCESS FOR MAKING BRIGHT YARNS**

[75] Inventors: **Pierre Allard, Calloux-Sur-Fontaines; Francois Buisson, Colmar, both of France**

[73] Assignee: **Rhone-Poulenc-Textile, Paris, France**

[22] Filed: **Aug. 2, 1972**

[21] Appl. No.: **277,163**

[30] **Foreign Application Priority Data**

Aug. 12, 1971 France ..... 71.29799

[52] **U.S. Cl. .... 260/78 TF; 264/184; 264/210 F**

[51] **Int. Cl.<sup>2</sup> ..... C08G 20/00; D01D 5/06**

[58] **Field of Search ..... 260/47 CB, 78 TF, 857 PI; 264/184**

[56] **References Cited**

UNITED STATES PATENTS

|           |        |                 |                  |
|-----------|--------|-----------------|------------------|
| 3,489,696 | 1/1970 | Miller          | ..... 260/857 PI |
| 3,528,937 | 9/1970 | Reynolds et al. | ..... 264/178 F  |
| 3,582,458 | 6/1971 | Haller          | ..... 260/857 PI |
| 3,673,160 | 6/1972 | Buisson et al.  | ..... 264/184    |

|           |        |                |                 |
|-----------|--------|----------------|-----------------|
| 3,708,459 | 1/1973 | Lubowitz       | ..... 260/78 TF |
| 3,717,696 | 2/1973 | Rochina et al. | ..... 264/205   |
| 3,733,308 | 5/1973 | Bach           | ..... 260/78 TF |

**FOREIGN PATENTS OR APPLICATIONS**

|           |        |        |               |
|-----------|--------|--------|---------------|
| 1,566,393 | 2/1967 | France | ..... 264/184 |
|-----------|--------|--------|---------------|

*Primary Examiner—Jay H. Woo*

*Attorney, Agent, or Firm—Stevens, Davis, Miller & Mosher*

[57]

**ABSTRACT**

A process is disclosed for making thermostable bright yarns by the wet-spinning of a solution in a polar organic solvent of a copolymer containing both amide-imide groups and amide-acid groups with a content of free COOH groups at least equal to 0.5 milliequivalent of acid per gram of copolymer, having an inherent viscosity of between 0.7 and 1.4 and obtained by reacting, at a temperature below 80°C solution of polyamideimide in a polar organic solvent, and a polyamide-acid prepolymer in solution in the same polar solvent, in proportions of 15 to 50, referred to the copolymer.

**9 Claims, No Drawings**

## PROCESS FOR MAKING BRIGHT YARNS

The present invention relates to a process for making bright yarns which are homogeneous and stable at high temperature by spinning a copolymer containing amide-imide linkages and imide linkages and to the filaments and fibers thus obtained.

A process is disclosed in U.S. Pat. No. 3,415,782 for making bright filaments having a base of polypyromellitiimide of good longitudinal and transverse strength by the dry-spinning of a solution of a polyamide-acid obtained from pyromellitic dianhydride and bis(amino-4-phenyl) ether or bis (amino-4-phenyl) sulfide and then transforming the polyamide-acid into polyimide by subsequently heating the resulting filaments. However, such a process has the disadvantage of being rather complicated technically because dry-spinning requires extensive apparatus and high evaporation-cell temperatures.

It is also known, from French Pat. No. 1,566,393, to 20  
prepare films by casting copolymers in solution ob-  
tained from a prepolymer containing amide and imide  
groups and a prepolymer containing imide groups and  
then heating to evaporate the solvent. However, the in- 25  
herent viscosities of these copolymers are low and gen-  
erally less than 0.5, which does not make it possible to  
obtain yarns of good quality.

The polyamide-imide yarns prepared by heretofore available wet-spinning processes are heterogeneous, lusterless and porous and therefore unsuitable for any textile use.

It has also been proposed to introduce linkages bearing alkaline sulfonate groups into polyamide-imide polymers to be spun into fibers but the presence of an alkaline metal is not always desirable.

It is therefore an object of this invention to provide a method for making bright yarns from polymers which contain both amide-imide linkages and imide linkages. Another object of the invention is to provide an improved wet-spinning process for making yarns from polymers having amide-imide and imide linkages. Still another object of the invention is to provide a bright, homogeneous, heat-stable yarn containing filaments prepared by wet-spinning a solution of a copolymer containing amide-imide and amide-acid linkages.

The foregoing objects and others are accomplished in accordance with this invention, generally speaking, by providing a process for making bright, homogeneous, heat-stable yarns by wet-spinning a solution of a copolymer having both amide-imide groups and amide-acid groups in a polar organic solvent therefrom into a solvent-non-solvent coagulating bath. The unreacted carboxyl groups in the copolymer should be equivalent to at least 0.5 acid milliequivalent per gram of dry copolymer. The inherent viscosity of the copolymer should be between 0.7 and 1.5. The copolymer may be prepared by reacting at a temperature of less than 80°C in a polar organic solvent, a polyamide-imide and a polyamide-acid containing reactive isocyanate groups. Preferably, the copolymer contains 15 to 50% polyamide acid. The spun copolymer after coagulation is drawn in air at room temperature, washed and dried by conventional methods and overdrawn at an elevated temperature. The dried product may be heat treated by a conventional method, if desired, before overdrawing.

A solution of copolymer having an inherent viscosity of between 0.7 and 1.5 which is suitable for wet-

spinning may be prepared in accordance with this invention by mixing a solution of polyamide-imide with a separately prepared fresh solution of polyamide-acid prepolymer but it is preferably prepared by forming the polyamide acid *in situ* in a solution of previously prepared polyamide-imide. The high viscosity of the copolymer tends to establish that a branched and/or sequential copolymer is obtained.

The polyamide-imide may be prepared by reaction in substantially stoichiometrical proportions in anhydrous polar organic solvent of at least one aromatic diisocyanate with an acid reagent formed of an aromatic acid anhydride and possibly a small proportion of an aromatic diacid, for example, up to 20% terephthalic acid or the like. The polyamide-imide obtained has the following amide-imide linkages:



and possibly amide linkages of the formula:



25 in which R represents an aromatic divalent radical,  $Ar_1$  represents a divalent aromatic radical, and  $Ar_2$  represents a trivalent aromatic radical having at least 6 carbon atoms.

Any suitable aromatic diisocyanate may be used. Preferred diisocyanates are 4,4'-diisocyanato-diphenylmethane, 4,4'-diisocyanatodiphenyl ether, 4,4'-diisocyanato-diphenyl propane, 2,4-toluylene diisocyanate, meta phenylene diisocyanate, para phenylene diisocyanate, 1,5-naphthylene diisocyanate and the like.

35 Suitable acid anhydrides include trimellitic anhydride and among the suitable aromatic diacids, terephthalic acid isophthalic acid, 4,4'-dicarboxy diphenyl methane, 4,4'-dicarboxy diphenyl ether, 4,4'-dicarboxy diphenyl sulfone, 4,4'-dicarboxy diphenyl benzophenone, 4,4'-dicarboxy diphenyl are particularly well suited.

The reaction takes place at a temperature which can range, for instance, from 80° up to 180°C and even more. A preferred method of preparation consists in gradually raising the temperature of the reaction medium, for instance, for 1 to 3 hours and then maintaining this temperature for a period of time which may vary from 1 to 4 hours.

50 The reaction takes place in an anhydrous polar organic solvent, preferably N-methyl pyrrolidone, so as to obtain a polymer concentration in the solution of between 18 and 35% by weight, and preferably between 22 and 28%, without taking into consideration a possible dilution at the end of the operation. The inherent 55 viscosity of the polyamide-imide obtained (measured in a 0.5% solution in N-methyl pyrrolidone at 25°C) is generally between 0.5 and 1.2 and generally close to 0.9.

60 The polyamide-acid prepolymer is obtained by reaction, in substantially stoichiometric proportions in the same organic solvent, of an aromatic diisocyanate (preferably the same as that used for preparing the polyamide-imide) with an acid reagent formed of a tetra-  
65 carboxylic acid dianhydride alone or mixed with the corresponding tetracarboxylic acid in the presence of a small amount of water, which may range up to about 3% by weight, based on the weight of solvent.

The starting temperature is generally between about 25° and about 40°C. It is preferably maintained within these limits for several hours. It is possible then gradually to increase the temperature without, however, going beyond 80°C, which would transform too many amide-acid groups into imide groups. The prepolymer then becomes insoluble. Its concentration in the solution is generally between 15 and 24%.

In the event that a previously prepared polyamide-imide is used — as is preferred — it is obviously necessary to cool it to less than 80°C and preferably to a temperature of between 25°C and 40°C before introducing the components of the polyamide-acid.

Among the tetracarboxylic acid dianhydrides mention may be made, for instance, of the pyromellitic and benzophenone 3,4,3',4'-tetracarboxylic dianhydrides. At the time that it is mixed with the polyamide-imide solution, the polyamide-acid solution must necessarily be freshly prepared (in the event that it is prepared separately) so that the polymer contains a maximum number of reactive isocyanate groups. In practice this solution must be used within 24 hours after its preparation.

The inherent viscosity of the polyamide-acid is generally of the order of about 0.4 to 0.5.

This value is not sufficient to permit wet-spinning under good conditions.

Under the conditions of the invention, there is obtained a copolymer whose inherent viscosity is generally greater than the inherent viscosity of the polyamide-imide and the polyamide-acid prepolymer used separately, which permits the wet-spinning of the solutions of the copolymer under good conditions.

The determination of the reactive isocyanate groups of the polyamide-acid leads to the assumption that a branched and/or sequential copolymer is formed by reaction of the isocyanate groups with mobile H functions of the polyamide-imide, since there is simultaneously noted an increase in the inherent viscosity of the copolymer obtained.

Moreover, the copolymer thus obtained has a content of free carboxyl groups greater than 0.5 (this content being expressed in milliequivalents per gram of dry copolymer). The best homogeneity and the best characteristics of the yarns are obtained with rates of free carboxyl groups at least equal to 0.6.

The proportions of polyamide-imide and polyamide-acid in the copolymer wet-spun in accordance with the present invention are between 50 and 85% polyamide-imide and 15 and 50% polyamide-acid based on the weight of copolymer. The preferred composition is 80% polyamide-imide and 20% by weight polyamide-acid.

The solvent may be any suitable polar organic solvent such as dimethyl acetamide, tetramethylene sulfone, or the like, preferably N-methyl pyrrolidone.

N-methyl pyrrolidone is poorly suited for the preparation of polyamide-acids of high molecular weight; on the other hand, it permits good reproducibility of the characteristics of the polyamide-imide and the polyamide-acid; surprisingly, copolymers of high molecular weight are obtained in this solvent. This is why N-methyl pyrrolidone constitutes the preferred solvent in the process claimed.

The spinning of the solution of the copolymer as described above is carried out in a coagulating bath composed essentially of solvent and non-solvent, generally at room temperature.

As non-solvent for the copolymer which can be used in the coagulating bath, mention may be made, for instance, of glycol, acetone, methylene chloride, although water is generally preferred for obvious reasons of economy.

The filaments are drawn, preferably in air, at a slow rate, and then washed, for instance on rollers, possibly with counter-current flow, and preferably with water, and dried, for instance on rollers, preferably at temperature of about 80° to 300°C. Thereupon the yarn is subjected to another drawing at elevated temperature, generally above 300°C, and possibly up to 400°C, and even beyond, by any means known to the man skilled in the art, for instance, in a tube or on a heating plate. Thus, in the copolymer, amid-acid groups are transformed into imid groups.

If it is desired to obtain filaments having particularly high mechanical properties, in particular excellent tenacity, one can effect a heat treatment before the last drawing, for instance at a temperature of between 200° and 300°C.

The yarns obtained, in addition to their brightness, have excellent physical and mechanical properties, and in particular good thermal stability and good non-inflammability.

The textile applications of the yarns thus obtained are extremely varied — protective clothing, equipment, conveyor belts, filtration of hot gases, etc.

The following examples in which the percentages are percentages by weight are given by way of illustration and not of limitation in order to illustrate the invention.

#### Example 1

There are prepared separately:

A. On the one hand, a polyamide-imide solution from a mixture of:

|                                    |        |
|------------------------------------|--------|
| 4,4'-diisocyanato-diphenyl methane | 875 g  |
| — trimellitic anhydride            | 672 g  |
| — N-methyl pyrrolidone             | 3349 g |

The polymer thus obtained has an inherent viscosity of 1.00 and has no free isocyanate groups.

B. On the other hand, a polyamide-acid solution from a mixture in stoichiometric proportions of:

|                                              |        |
|----------------------------------------------|--------|
| 4,4'-diisocyanato-diphenyl methane           | 250 g  |
| — pyromellitic dianhydride                   | 218 g  |
| — N-methyl pyrrolidone containing 0.8% water | 1730 g |

There is obtained a prepolymer of an inherent viscosity of 0.40, having a content of isocyanate groups of 1.83 (expressed in milliequivalents per gram of dry prepolymer) and a content of carboxylic groups of 3.77 (expressed in milliequivalents per gram of dry prepolymer).

The two solutions A and B are mixed in different proportions so as to obtain C, D, E, F, G containing 10, 15, 20, 35 and 50% respectively of polyamide-acid prepolymer.

The determination of the isocyanate groups on the prepolymer and the copolymer is effected immediately after the reaction by potentiometry at room temperature in dimethyl acetamide. After the determination on the copolymer there is noted the practically complete disappearance of the isocyanate groups (see Table I).

The respective concentrations of polymers C, D, E, F, G in N-methyl pyrrolidone are 21.9, 22.2, 22.1, 18 and 19.2% respectively; thereupon each of the solutions is spun separately through a spinneret of 64 holes of a diameter of 0.05 mm into a coagulating bath containing 60% N-methyl pyrrolidone and 40% water, maintained at room temperature.

The filaments are then washed with water in counter-current, at room temperature, and then dried on rollers at 80°C and then at 170°C, drawn at room temperature, at rates given in Table I below. They are then heat treated in an oven for 2 hours at 240°C and drawn again at 420°C in a tube at rates indicated in Table I below, which sets forth the characteristics of the polymers and of the yarns obtained.

TABLE I

| COPOLYMERS                             | C                                       | D            | E              | F            | G            |
|----------------------------------------|-----------------------------------------|--------------|----------------|--------------|--------------|
| Inherent viscosity<br>m.eq.isocyanates | 0.93<br>trace, not<br>determin-<br>able | 0.95<br>0.14 | 1.32<br>0.20   | 1.14<br>0.17 | 0.94<br>0.24 |
| COOH groups, meq.                      | 0.40                                    | 0.6          | 1.01           | 1.52         | 2            |
| Drawing-air: rate                      | 1.6                                     | 1.5          | 1.85           | 1.7          | 1.5          |
| Overdrawing: rate                      | 4.38                                    | 4.69         | 3.70           | 3.40         | 3.27         |
| Count dtex                             | 99                                      | 77           | 117            | 121          | 101          |
| Resistance g/tex                       | 24                                      | 33.6         | 39.4           | 34.2         | 35.5         |
| Elongation, %                          | 11                                      | 12.3         | 10.9           | 10.7         | 10.7         |
| Appearance of the<br>yarn              | dull and<br>irregular                   | bright       | very<br>bright | bright       | bright       |

It is noted that the yarns obtained from copolymers D, E, F, G are bright, contrary to the yarn obtained from copolymer C the content of COOH groups of which is insufficient.

The heat stability of sample E was evaluated by the loss of strength upon aging, as follows:

— for 300 hours at 177°C: — 12.4%  
— for 1000 hours at 177°C: — 60.5%

## Example 2

A polyamide-imide is prepared from:

— diisocyanato-4,4'-diphenyl ether 630 g  
— trimellitic anhydride 480 g  
— N-methyl pyrrolidone 2818 g

The polymer obtained has an inherent viscosity of 1.05.

There is introduced into the previously prepared polyamideimide solution, cooled to 38°C:

— diisocyanato-4,4'-diphenyl ether 32 g  
— pyromellitic dianhydride 27.7 g  
— N-methyl pyrrolidone 104 g  
— water 1.37 g

During the course of 2 hours, 190 g of N-methyl pyrrolidone and 1.37 g of water are added at 38°C, maintaining this temperature for 1 hour, whereupon the temperature is increased to about 60°C, which temperature is maintained for another hour. Prepared separately, the prepolymer has an inherent viscosity of 0.53. The copolymer obtained, which has an inherent viscosity of 1.39 and a content of carboxylic acid groups of 0.78 is spun in solution in N-methyl pyrrolidone at a

concentration of 23.1% through a spinneret of 64 orifices of a diameter of 0.05 mm into a coagulating bath composed of N-methyl pyrrolidone and water, in a proportion of 60:40, at room temperature.

The yarn obtained is washed with water on rollers at room temperature, and then dried on two drying rollers of a temperature of 80° and 170°C respectively.

After drawing in air at a rate of 1.22, the yarns undergo a second drawing in a tube at 400°C, at a rate of 2.50.

10 The properties of the yarns are as follows:

|    |                                               |              |
|----|-----------------------------------------------|--------------|
| 15 | Count                                         | 446 dtex     |
|    | Dry strength in g/tex                         | 43           |
|    | Elongation, dry %                             | 8.2          |
|    | Aging:<br>after 300 hours at 177°C            | +9.4%        |
|    | Loss of Strength<br>after 1000 hours at 177°C | -34%         |
|    | Appearance                                    | very bright. |

Although the invention has been described in detail for the purpose of illustration, it is to be understood that such detail is solely for that purpose and that variations can be made by those skilled in the art without departing from the spirit and scope of the invention except as it may be limited by the claims.

We claim:

25 1. A method for making a non-inflammable heat-stable, bright yarn comprising

1. wet-spinning into a coagulating bath a solution in a polar organic solvent of a copolymer which contains both amide-imide groups and amide-acid groups, the free carboxyl group content of the copolymer being at least equal to 0.5 milliequivalents of acid per gram of dry copolymer, said copolymer having an inherent viscosity of between 0.7 and 1.5, said copolymer having been prepared by reacting in a polar organic solvent at a temperature below 80°C a polyamide-imide and a polyamide-acid prepolymer;

2. drawing the resulting filaments in air at ambient temperature;

3. washing and drying; and

40 4. overdrawing the product at an elevated temperature.

2. The method of claim 1 wherein the copolymer contains from 15 to 50% polyamide-acid.

3. The method of claim 1 wherein the washed and dried filaments are heat treated prior to overdrawing.

45 4. The method of claim 1 wherein the solvent in the spinning solution and the coagulating bath is N-methyl pyrrolidone.

5. The method of claim 1 wherein the polyamide-acid is prepared in a solution containing the polyamide-imide solution.

6. The method of claim 1 wherein the polyamide-imide is the reaction product of an aromatic diisocyanate and trimellitic anhydride and the polyamide-acid is the reaction product of an aromatic diisocyanate and pyromellitic dianhydride.

55 7. The method of claim 5 wherein the diisocyanate used in each reaction is 4,4'-diphenylmethane diisocyanate.

8. The method of claim 1 wherein an aromatic dicarboxylic acid is included in the preparation of the polyamideimide.

9. A non-inflammable, heat-stable, bright yarn prepared by the method of claim 1 from a copolymer which contains both amide-imide groups and amide-acid groups, said copolymer having a free carboxylic group content which is at least equal to 0.5 milliequivalents of acid per gram of dry copolymer and having an inherent viscosity of between 0.7 and 1.5.

\* \* \* \*